

Nov. 22, 1966

A. ELMENDORF

3,287,203

HARDWOOD FLOORING

Filed March 14, 1962

2 Sheets-Sheet 1



FIG. 2.



FIG. 2a.



INVENTOR.  
Armin Elmendorf,  
BY Parker & Carter  
Attorneys.

Nov. 22, 1966

A. ELMENDORF

3,287,203

HARDWOOD FLOORING

Filed March 14, 1962

2 Sheets-Sheet 2



INVENTOR  
Armin Elmendorf,  
BY Parker & Carter  
Attorneys.

## 1

3,287,203

## HARDWOOD FLOORING

Armin Elmendorf, Palo Alto, Calif., assignor to Elmendorf Research Incorporated, a corporation of California

Filed Mar. 14, 1962, Ser. No. 179,709  
3 Claims. (Cl. 161—123)

This invention is in the field of flooring, particularly an improved hardwood flooring which is resistant to denting, and is a continuation-in-part of my copending application Serial No. 100,659, filed April 4, 1961 now abandoned.

A primary purpose of the invention is a hardwood flooring in which the resistance to denting is greater than that of the wood itself.

Another purpose is a hardwood flooring which does not have to be refinished during its lifetime.

Another purpose is a hardwood flooring which provides the traction of vinyl tile flooring.

Other purposes will appear in the ensuing specification, drawings and claims.

The invention is illustrated diagrammatically in the following drawings wherein:

FIGURE 1 is a perspective of a partially laid floor which embodies the principles disclosed herein,

FIGURE 2 is a partial section through one of the flooring squares of FIGURE 1,

FIGURE 2a is a partial section through a modified flooring square, and

FIGURES 3-5 are graphs illustrating the principles upon which this invention is based.

Most of the hardwood flooring installed in homes in the United States today is made of oak, although maple is also used to a substantial extent for gymnasium and commercial floors where eye appeal is of secondary importance. From the point of view of eye appeal, walnut, mahogany, and a number of tropical woods are frequently preferred to oak, but they are all deficient in hardness and are generally not regarded as satisfactory for flooring for that reason. Experience in the manufacture of walnut and mahogany flooring has demonstrated that such floors dent easily in service and being expensive, marring through denting rapidly depreciates the floor. Denting of soft wood flooring made of vertical grain lumber is also a serious drawback to the extensive use of soft wood such as hemlock, pine and Douglas fir for flooring. Oak floors also dent in service, such dents resulting from nails and heels of shoes, pointed heels of ladies' shoes, rolling of furniture and prolonged pressure from furniture casters. While oak floors do not dent as readily as the softer woods, such as walnut and mahogany, the presence of dents is an indication that the floor must be refinished in time by machine sanding and refinishing. It is for this reason that hardwood floors always call for a minimum thickness in the wearing layer of  $\frac{1}{8}$  inch. In the case of hardwood plywood flooring, the top ply must be at least  $\frac{1}{8}$ -inch thick to provide the necessary durability for prolonged service.

Wood floors are available in various types. They may be in the form of strips with tongue-and-groove or square edges, the latter being nailed to the sub-floor and generally finished on the job. In another form, the wood is used in the form of square blocks, each consisting of several slats, the slats of one block being at right angles to those of the adjacent blocks. The flooring squares may

## 2

also be in the form of plywood having  $\frac{1}{8}$ -inch veneer faces.

Many different finishing schedules are commonly used on hardwood flooring, such as shellac followed by waxing, shellac plus varnish, or several coats of varnish, or penetrating sealers in combination with wax. In most floor finishes the finish has a thickness ranging from one to three mills (.001-.003 inch). For home use where the floor is subjected to normal wear, the thickness of the varnish coat generally falls within this range. It is customary after several years of use when the finish begins to wear off, to sand the floor and refinish it. Experience has shown that the wood must be at least  $\frac{1}{8}$ -inch thick to meet this requirement. This minimum thickness is therefore often a requirement in flooring specifications. In the case of penetrating sealer finishes, additional applications of the sealers are sometimes resorted to as the floor wears, but the major resistance to wear is provided by the wood itself. This is also true of wax finishes.

20 A main purpose of the present invention is to produce a hardwood floor so made that it does not dent readily, and so finished that the inconspicuous denting of the finish which does take place in time is not objectionable, and so durable that it never wears through during the life of the floor. The wear resistance of the wood itself is never called upon in service. Such finishing becomes possible when the resistance to indentation exceeds that of the natural wood. Printed or wood grain reproductions are not acceptable. The natural wood must be used to 25 get the color and grain variations and the "flash" that only natural wood provides.

Many attempts have been made to harden wood by compression and by impregnation, but the effect of such hardening has been either to embrittle the wood, thereby 30 reducing its wear resistance, or to make it so hard that it is slippery when waxed and therefore dangerous to walk on. Excessive hardness is therefore not acceptable.

I have now found that, contrary to accepted theory, under certain conditions, the resistance to indentation of 35 hardwood floors may be increased by reducing the thickness of the wood. I have found that in combining a very thin layer of natural wood with a hard ligno-cellulosic base, if the thickness of the natural wood is reduced, a thickness will be reached at which the resistance to indentation exceeds that of conventional flooring made of 40 this wood, and if thin enough the resistance to indentation may even exceed that of the base to which the wood is bonded. This result is achieved without impregnating the wood or changing its structure, composition or density.

I have found that Douglas fir plywood and normal 45 particle boards which are generally used as underlays for flexible floor coverings are not satisfactory substrates for my purpose. They lack the necessary hardness. The density of underlays generally ranges from 0.45 to 0.70. I have found that wood fiber hardboards such as tempered Masonite and equivalent products have the necessary hardness and toughness to produce the results desired. The density of satisfactory wood fiber hardboard substrates ranges from about 0.85 50 to 1.15. Other ligno-cellulosic boards, such as certain high density shaving or particle boards are also suitable base materials and adequately hard when their density lies in this range. Cement-asbestos boards of the high density type also have the necessary hardness, dent-resistance, and dimensional stability.

The present invention relates to a wood flooring of

the same general thickness as vinyl flooring, namely,  $\frac{1}{12}$  inch to  $\frac{1}{8}$  inch. It is sufficiently durable and dent resistant, and is sufficiently pliable so that it can be laid with conventional flooring adhesives using manually applied momentary pressure. This is a requirement of major importance in the field of flooring. In a thickness comparable with vinyl tile, my flooring is sufficiently flexible so that it follows the contour of the subfloor, but, unlike vinyl tile, it does not telegraph the wood grain of the plywood subflooring or underlayment or joints in the same. The present flooring requires no edge leveling means such as a tongue-and-groove connection, and it can be laid with the same procedure and speed as conventional asphalt or vinyl tile. This is a surprising result in view of the unbalanced construction of the flooring. Due perhaps to the thinness of the wood, the slight deviations from flatness that may occur are never serious and do not prevent satisfactory bonding.

When this floor is to be laid over a wood plank subfloor, an underlayment must be used as with flexible floor coverings such as asphalt tile or vinyl tile. Inasmuch as Douglas fir plywood is one of the commonest underlayment materials, one of the requirements of this improved flooring consists in the necessity for being able to use it successfully on Douglas fir plywood underlayment or subflooring. Experience in the application of vinyl tiles to plywood subflooring or to plywood underlayment has shown that the nails used in the installation of the plywood and the joints between the sections of plywood, as well as surface roughness due to grain raising, will all telegraph through the vinyl tile, thereby detracting greatly from the appearance of the floor. This is generally regarded as one of the major liabilities of vinyl tile flooring. I have found that no such telegraphing of joints, nail heads or surface roughness takes place through my improved thin wood flooring of the same thickness as vinyl flooring. The thin hardwood flooring of this invention is sufficiently flexible so that it follows the contour of the subfloor and successfully bridges joints in the same without telegraphing.

The floor tile must be sufficiently flexible so that the pull or tack exerted by conventional flooring adhesives is adequate to hold the flooring in contact with the subfloor while the adhesive sets. I have found that in order to obtain over-all bonding the thickness of the high density hardboard base should not be greater than about  $\frac{1}{8}$  inch and preferably should be about  $\frac{1}{12}$  inch. If the base is appreciably thicker than about  $\frac{1}{8}$  inch, some difficulty may be experienced due to the springing away from the subfloor at tile edges while the adhesive is still fresh and edge support as by means of splines becomes necessary.

In FIGURE 1, the plywood subflooring is indicated at 10 and the flooring at 12. The floor tile disclosed consists of a substrate or base 14, preferably of the wood-fiber hardboard or high-density shaving or particle board type described. A natural wood layer 18 is suitably bonded to the base and is of a thickness as described hereinafter. Covering the natural wood layer 18 is a film 16 which is of a clear abrasion-resistant material so that the grain of the natural wood will be visible. The layer 16 will be described hereinafter.

FIGURE 3 illustrates the results of tests made to determine the optimum thickness of the hardboard base 14. Indentation tests were made using a  $\frac{1}{16}$ -inch steel ball and a pressure of 150 pounds on the ball, on a tempered hard board, having a specific gravity of 1.10, bonded to  $\frac{3}{8}$ -inch Douglas fir plywood. The indentation shown in the graph is the residual indentation two hours after removal of the pressure. A pressure of 150 pounds on the steel ball corresponds to the weight of an average person. The test results indicate that indentation progressively increases with the reduction of thickness of the base until a thickness of about  $\frac{1}{20}$  inch

is reached at which point the steel ball breaks through. The base must therefore not be thinner than about  $\frac{1}{20}$  inch. As stated earlier in order to retain the necessary degree of flexibility, the maximum thickness of the base should not exceed about  $\frac{1}{8}$  inch, with  $\frac{1}{2}$  inch being a preferred thickness.

The maximum thickness of the base is determined by the desired flexibility or suppleness of the flooring. The flooring may also be made supple by cutting grooves 20 in the back as shown in FIGURE 2a. These grooves may be V-shaped or rectangular or of any other shape provided their depth is adequate. Grooves are frequently cut in wood flooring where they serve as a means for escape of the adhesive squeezed out in laying the floor. I may use grooves in order to improve the suppleness. For this reason my grooves must be deep enough to achieve this result. Superior suppleness results when the thickness of the base at the bottom of the grooves, indicated at 22, is about  $\frac{1}{20}$  inch, but some improvement in flexibility is obtained even when the grooves are shallower and the thickness at the base is somewhat greater than  $\frac{1}{20}$  inch.

FIGURE 4 illustrates the residual indentation in indentation tests made on walnut veneer bonded to  $\frac{1}{8}$ -inch tempered hardboard when the hardboard is bonded to  $\frac{3}{8}$ -inch Douglas fir plywood underlayment. A  $\frac{1}{16}$ -inch diameter steel ball was placed on the laminate and subjected to a pressure of 150 pounds. The curve shows the residual indentation two hours after removal of the pressure for various thicknesses of veneer. There was no change in the residual indentation after two hours. It appears from these tests that the residual indentation was reduced by reducing the veneer thickness if the veneer is bonded to a base that is substantially harder than natural wood, such as temperer hardboard.

The results shown in FIGURE 4 suggest that a veneer as thin as  $\frac{1}{100}$  inch could be used if no other factors, such as adhesive strike-through, had to be considered.

It will be noted from FIGURE 4 that when the veneer is bonded to hardboard as described and the thickness of the veneer is about .04 inch, the depth of the residual indentation is .02 inch, about the same as that on a  $\frac{1}{8}$ -inch hardboard base alone (FIGURE 3). When the veneer thickness is less than about .04 inch, the depth of indentation is, surprisingly, even less than that of  $\frac{1}{8}$ -inch hardboard alone. On the other hand, when the thickness of the veneer exceeds about .04 inch, the depth of the residual indentation progressively increases and is greater than the indentation of the  $\frac{1}{8}$ -inch hardboard alone. For this reason, it is preferable to limit the veneer thickness to about .04 inch. In this way, the resistance to denting of the hardboard base is utilized to its fullest extent. This same result is pointed up in FIGURES 7 and 8 of copending application Serial No. 100,659, which show the indentation at 150 pounds of pressure when veneers of various thicknesses are bonded to  $\frac{1}{4}$ -inch hardboard.

Several synthetic products, such as the polyvinyl chlorides, polyurethanes, and epoxy resins possess the wear resistance required in my flooring if applied in a thickness of at least .005 inch. Under foot traffic, finishes made of these products yield sufficiently to provide good traction. They are generally softer than hardwood such as oak. The finish or surface layer 18 may be applied in the form of a liquid or in the form of a film of appropriate thickness. Preferably the thickness of the finish 18 is at least five times as thick as conventional floor finishes, bonded to the wood. In order to be sufficiently durable, and to prevent the wearing of the wood layer 18, this film must be at least .005 inch in thickness, and it must possess a traction comparable to that of vinyl floor tile. Such products yield considerably under pressure so that they dent noticeably if they are thicker than .030 inch. I have found that a coating of clear vinyl resin comparable in physical properties with the clear resin used for vinyl floor tile may

be used with a thickness limitation ranging from about .005 inch to .030 inch.

The entire assembly including the hardboard base, the wood layer and the surface layer are suitably bonded together in a press using pressing conditions in common use for each bond.

FIGURE 5 shows the results of indentation tests made on several types of commercial flexible floor tile. These tile were all about  $\frac{1}{8}$ -inch thick and were tested for dent resistance. All of the tests were made with a steel ball  $\frac{3}{16}$ -inch in diameter and an applied pressure of 150 pounds. The diagrams illustrate the depth of indentation of each product at a load of 150 pounds, immediately after releasing pressure, one hour after release of pressure, and 24 hours after release of pressure. The tests included hardboard, particle board, oak and maple wood, vinyl tile, both of the solid color type and clear, vinyl asbestos tile, asphalt tile, rubber tile and two tile made from oak and in accordance with this invention. The results shown in the bar diagrams of FIGURE 5 illustrate that commercially-made vinyl tile are relatively soft and dent easily, but on the other hand they recover well. This is particularly true of clear vinyl of the type used for the surface film 18. Vinyl asbestos and asphalt tile dent less under load and recover less than vinyl tile. Rubber tile dents easily and does not recover as well as vinyl of the clear type. The diagrams also show that tempered hardboards dent less than vinyl tile. The same applies to high density particle board. Such flooring woods as white oak and hard maple dent more than tempered hardboard, or high density particle board and recover little.

The most surprising results of the tests are illustrated in the bars at the right of FIGURE 5, from which it will be seen that typical floorings of this invention dent less than flooring hardwood such as oak and maple and that the residual dents after 24 hours are no greater than those of clear vinyl tile. Since one of the major advantages of vinyl tile as a flooring material is its recovery from indentation, the product of this invention is comparable in this property to vinyl tile even though it is much harder and suffers less immediate indentation.

Wear tests were made simulating the abrasion suffered by flooring subjected to heavy foot traffic. Observations frequently made have shown that wood floor finishes wear through first at the locations where persons walking on the same change their direction as, for example, at the foot of a stairway or at entrances to doorways. Such tests must be made at pressures corresponding to those of foot traffic and must simulate the abrasion of shoe leather on dusty floors. Such tests were conducted on typical hardwood floors factory-finished by two well-known manufacturers of hardwood flooring. Similar wear tests were made on products of this invention using a clear vinyl film in a thickness of 12 mils and of a hardness comparable to that of the clear vinyl tile illustrated in FIGURE 5. It was found that the thickness of the finish was reduced less than one mil in the time required for complete destruction of the conventional floor finishes applied by wood flooring manufacturers. On this basis it is to be expected that a vinyl film five mil in thickness will wear at least five times as long as standard hardwood floor finishes. It may be further concluded that a vinyl film finish thicker than five mil will not wear through for the life expectancy of floors made as disclosed herein. In other words, in actual service the wood in the tile of this invention is never subjected to wear.

The results of tests shown in FIGURES 3, 4 and 5, and FIGURES 7 and 8 of copending application Serial No. 100,659, indicate that the product of this invention is at least as dent resistant as the base material, or tempered hardboard. The base material in turn is harder than common flooring hardwoods, such as white oak and hard maple. Most flooring hardwoods are in turn harder than vinyl floorings.

The flooring tiles of this invention are suitable for

bonding to a subfloor or underlayment with conventional flooring adhesives using momentary pressure. There are no tongue-and-groove joints or splines to align the edges and to bring the tile surfaces to the same level. The flooring consists of a single layer of very thin natural wood bonded to a base that is harder than flooring hardwood and that has a thickness of not less than  $\frac{1}{20}$  inch nor greater than  $\frac{1}{8}$  inch. The layer of natural wood, for example oak or walnut is preferably thinner than .04 inch. The thin natural wood is bonded to such a base and is faced with a wear-resistant transparent film comparable in hardness and durability to clear vinyl used for floor tile, and which is softer than flooring hardwood to obtain satisfactory traction.

Although the invention has been generally described as suitable for forming flooring tiles, it should be realized that flooring planks may also be formed by following the disclosure herein.

Whereas the preferred form of the invention has been shown and described herein, it should be realized that there are many modifications, alterations and substitutions thereto within the scope of the following claims.

I claim:

1. A prefinished wood flooring having a dent resistance exceeding that of flooring hardwood and which flooring is adapted for bonding to a subfloor by pressure momentarily applied and which flooring requires no refinishing after installation, including,

a ligno-cellulosic fibrous base having a hardness resulting due to a density of from about 0.85 to 1.15, said base having a thickness between about  $\frac{1}{8}$  inch and  $\frac{1}{20}$  inch to provide serviceability under extended use together with adequate flexibility to allow said base to follow the undulations in a subfloor when bonded to a subfloor with an adhesive while using momentary pressure,

a layer of hardwood veneer, thinner than about 0.04

inch, said veneer bonded to said base,

and a clear wear resistant covering bonded to the

veneer, said covering consisting essentially of a resin

film having flexibility and softness sufficient to pro-

vide adequate traction for the installed flooring, and

said film having a thickness of at least 0.005 inch.

2. A prefinished wood flooring having a dent resist-

ance exceeding that of flooring hardwood and which

flooring is adapted for bonding to a subfloor by momen-

tarily applied pressure and which flooring requires no re-

finishing after installation, including,

a ligno-cellulosic fibrous base having a hardness re-

sulting due to a density of from about 0.85 to 1.15,

said base having a thickness between about  $\frac{1}{8}$  inch

and  $\frac{1}{20}$  inch to provide serviceability under ex-

tended use together with adequate flexibility to allow

said base to be bonded to a subfloor with an adhesive

while using momentary pressure,

a layer of hardwood veneer, thinner than about 0.04

inch, said veneer bonded to said base,

a clear wear-resistant covering bonded to the veneer,

said covering consisting essentially of a vinyl resin

film having flexibility and softness to provide ade-

quate traction for the installed flooring.

3. A prefinished wood flooring having a dent resist-

ance exceeding that of flooring hardwood, which flooring

is adapted for bonding to a subfloor by pressure momen-

tarily applied, and which flooring further requires no re-

finishing after installation, including,

a ligno-cellulosic fibrous base having a hardness com-

parable to commercial hardboard, the bottom of said

base having grooves therein to improve the supple-

ness of the flooring, the thickness of the base at the

bottom of the grooves being about  $\frac{1}{20}$  inch,

a layer of natural wood veneer, thinner than about 0.04

inch, said veneer bonded to the top of said base,

a clear wear resistant covering bonded to the veneer,

said covering consisting essentially of a vinyl resin film having flexibility and softness sufficient to provide adequate traction for the installed flooring, and said vinyl resin film having a thickness of at least 0.005 inch.

5

|           |         |            |           |
|-----------|---------|------------|-----------|
| 2,850,890 | 9/1958  | Rubenstein | 52—229    |
| 2,896,682 | 7/1959  | Elmendorf  | 161—123 X |
| 2,932,596 | 4/1960  | Rayner     | 161—165   |
| 2,989,420 | 6/1961  | Zdanowski  | 117—176   |
| 3,108,030 | 10/1963 | Taylor     | 161—268 X |

## References Cited by the Examiner

## UNITED STATES PATENTS

|           |         |           |           |
|-----------|---------|-----------|-----------|
| 2,054,869 | 9/1936  | Smolak    | 161—251   |
| 2,067,012 | 1/1937  | Loetscher | 161—268 X |
| 2,181,164 | 11/1939 | Alexander | 287—20.92 |
| 2,220,898 | 11/1940 | Franklin  | 287—20.92 |
| 2,758,044 | 8/1956  | Terry     | 52—510 X  |
| 2,831,793 | 4/1958  | Elmendorf | 161—114   |

## FOREIGN PATENTS

|         |      |         |
|---------|------|---------|
| 770,802 | 1934 | France. |
|---------|------|---------|

RICHARD W. COOKE, JR., *Primary Examiner.*JACOB L. NACKENOFF, *Examiner.*WILLIAM I. MUSHAKE, J. E. MURTAGH,  
*Assistant Examiners.*